

# United States Patent [19]

## Bryant

[11] Patent Number: 4,856,299

[45] Date of Patent: Aug. 15, 1989

- [54] KNITTED FABRIC HAVING IMPROVED  
ELECTRICAL CHARGE DISSIPATION AND  
ABSORPTION PROPERTIES

[75] Inventor: Kenneth G. Bryant, Charlotte, N.C.

[73] Assignee: Conductex, Inc.

[21] Appl. No.: 132,122

[22] Filed: Dec. 14, 1987

#### **Related U.S. Application Data**

- [63] Continuation-in-part of Ser. No. 940,864, Dec. 12, 1986.

- [51] Int. Cl.<sup>4</sup> ..... D04B 7/16  
[52] U.S. Cl. ..... 66/202; 66/195;  
139/425 A  
[58] Field of Search ..... 66/202, 192, 190, 193,  
66/195; 139/425 A; 420/242; 57/901; 361/210,  
212; 174/117 M

[56] References Cited

U.S. PATENT DOCUMENTS

- |           |         |                    |         |
|-----------|---------|--------------------|---------|
| 2,845,962 | 8/1958  | Bulgin .....       | 139/420 |
| 3,011,172 | 12/1961 | Tames .....        | 2/51    |
| 3,288,175 | 11/1966 | Valko .....        | 139/425 |
| 3,422,460 | 1/1969  | Burke et al. ..... | 2/73    |

- |           |         |                          |           |
|-----------|---------|--------------------------|-----------|
| 3,582,448 | 6/1971  | Okuhashi et al. ....     | 161/87    |
| 3,586,597 | 6/1971  | Okuhashi .....           | 161/87    |
| 3,699,590 | 10/1972 | Webber et al. ....       | 2/73      |
| 3,764,097 | 10/1973 | Matthews et al. ....     | 244/142   |
| 3,806,959 | 4/1974  | Gross .....              | 5/334 R   |
| 3,986,530 | 10/1976 | Maekawa .....            | 139/425 R |
| 4,232,082 | 11/1980 | Noritake .....           | 428/225   |
| 4,335,589 | 6/1982  | Flasher .....            | 66/202    |
| 4,398,277 | 8/1983  | Christiansen et al. .... | 361/220   |
| 4,422,483 | 12/1983 | Zins .....               | 139/420 R |
| 4,475,141 | 10/1984 | Antonevich .....         | 361/220   |
| 4,557,968 | 12/1985 | Thornton et al. ....     | 428/229   |
| 4,590,623 | 5/1986  | Kitchman .....           | 2/85      |
| 4,606,968 | 8/1986  | Thornton et al. ....     | 428/229   |
| 4,753,088 | 6/1988  | Harrison et al. ....     | 66/202    |

*Primary Examiner*—Ronald Feldbaum  
*Attorney, Agent, or Firm*—Kenyon & Kenyon

[57] ABSTRACT

A knitted fabric having improved electrical charge dissipation, absorption, stain resistance, anti-pilling and linting and tensile strength properties, constructed so as to form a conductive matrix capable of discharging an electrical charge along any direction of the course and wale of the fabric.

**11 Claims, 3 Drawing Sheets**



Fig. 1.





Fig. 3.



**KNITTED FABRIC HAVING IMPROVED  
ELECTRICAL CHARGE DISSIPATION AND  
ABSORPTION PROPERTIES**

This is a continuation-in-part application of U.S. application No. 940,864, filed Dec. 12, 1986.

**BACKGROUND OF THE INVENTION**

**1. Field of the Invention**

This invention relates to a new and improved knitted fabric having improved electrical charge dissipation, absorption, stain resistance, anti-pilling and linting and tensile strength properties. More specifically, this invention relates to a readily manufactured knitted fabric comprised of nonconductive yarn that extends along the wale and combined with conductive fibers that form overlaps and underlaps within the nonconductive knit to such an extent so as to form a combined stitch construction, e.g., a modified "Queen's Cord" construction, providing an electrically conductive matrix capable of quickly dissipating charge along any direction of both the course and wale. Still further, the invention's construction provides increased absorption, stain resistance and tensile strength properties, and minimizes pilling and linting.

**2. Description of the Prior Art**

Electrostatic charge accumulates on clothing as the wearer moves his or her arms and legs and as he or she walks on non-conductive floor surfaces. The accumulation of such static charge creates a problem in tight-fitting garments such as hosiery and sporting apparel in which static charge causes adjacent garments to cling to one another. This static cling causes both discomfort for the wearer and unpleasant shocks. Such charge accumulation can also pose significant problems when the wearer works in an environment in which any static charge is undesirable or dangerous. A need exists, therefore, for a means to control electrostatic charge accumulation on fabric, particularly fabric used in clothing worn by individuals who occupy or handle materials in areas in which an electrostatic discharge can be hazardous to the individual or can damage material which is being handled by the wearer, e.g., in hospital environments where potentially explosive gases are present and patient comfort is important, or in "clean rooms" where electrically sensitive microcircuits are manufactured.

Still further, those environments, particularly hospitals, in which the control of electrostatic charge accumulation is important require a fabric, including particularly a towel, that can provide a multitude of functions and uses. In addition to control of electrostatic discharge, improved absorbancy, stain resistance and tensile strength, as well as minimized pilling and linting, are important characteristics for fabrics used in hospital environments. The advantages of use of this invention in other environments are also evident.

The utilization of fibers possessing electrical conductivity (e.g., metal fibers, fibers coated with electrically conductive material, or metal laminate filaments) in combination with common natural and manmade fibers to produce a woven, knitted, netted, tufted, or otherwise fabricated structure, which readily dissipates static charge as it is generated is well known.

In U.S. Patent 3,823,035, issued to Sanders, an electrically-conductive textile fiber is disclosed in which finely-divided electrically conductive particles are uniformly suffused in a filamentary polymer substrate.

Sanders discloses the interweaving of such electrically conductive fibers with ordinary threads made from natural fibers such as cotton or wool in an amount sufficient to render the electrical resistance of the fabric to a value of  $10^9$  ohms/cm.

U.S. Pat. No. 4,312,913, issued to Rheaume, discloses a heat-conductive woven fabric comprising a plurality of fill layers of weavable yarns, each yarn comprising a plurality of fibers that are metallic or are coated with an effective amount of a metallic, heat conducting material. An angle weave pattern is woven through the layers of fill yarns in Rheaume, and this angle woven pattern extends from the top to the bottom of several layers of fill yarns.

Similarly, U.S. Pat. No. 4,296,855, issued to Blalock, also discloses a woven pattern of filler and warp yarns comprised of an electrically insulating material suffused with electrically conducting carbon particles, the warp and filler being woven in an open mesh configuration.

U.S. Pat. No. 4,422,483, issued to Zins, discloses a multiplicity of elongated filaments which are essentially parallel to each other and which form a single ply of a conductive thread for woven fabrics. The elongated filaments in Zins are non-textured continuous, non-conductive filaments or warp threads which are combined together with conductive filaments or fill threads to form a conductive woven fabric.

Neither Sanders, Rheaume, Blalock or Zins disclose a conductive knitted fabric. While U.S. Pat. No. 4,443,515, issued to Atlas, and its divisional 4,484,926, disclose that conductive fibers comprised of synthetic polymers may be incorporated into knitted fabrics, those references do not disclose a pattern whereby such conductive fibers can be economically incorporated into a knitted fabric so as to dissipate static electricity in any direction along the course and wale directions of the fabric. Nor do they have the special combination of elements, including improved absorption, stain resistances and tensile strength and minimized pilling and linting, unique to this invention.

U.S. Pat. No. 4,398,277, issued to Christiansen et al., does disclose a pattern whereby insulative yarn and electrically conductive yarn are knitted together on two levels. The insulative yarn in Christiansen et al. forms a series of interlocking loops on both the technical face and back of the fabric in a tricot construction, while the electrically conductive yarn forms a series of chain stitches on only the technical face. Christiansen et al. disclose that when their fabric is knitted in such a two layer construction, one of the surfaces (i.e., the technical face) will be relatively nonconductive. Electrical charge dissipation in such a construction, therefore, is limited to the wale direction of the technical face of the fabric.

Attempts have been made to develop a knitware pattern that can be economically manufactured, which require the use of a relatively small amount of conductive fiber and which possess electrical conductivity along both the course and wale directions and on both the technical face and back of a two layer knitted fabric. A knitted fabric in which conductive yarn is knitted in an argyle pattern together with nonconductive yarn, resulting in a fabric having electrical conductivity along the course and wale directions on both the technical face and back, has been constructed.

The argyle construction suffers from several disadvantages. Such a construction requires that the conductive fiber be stitched simultaneously along both the

course and wale directions to form a saw-tooth pattern known as an "Atlas stitch" which, when joined to a similar adjacent stitch, forms the argyle pattern. Such simultaneous horizontal and vertical movement of fiber requires that the argyle knit be manufactured on a knitting machine having at least two separate guidebars dedicated to the argyle construction. Further, the argyle construction requires the use of a substantial amount of conductive yarn, which is a significant disadvantage given that such yarn is currently more than about thirty-six times as expensive as nonconductive yarn. An additional significant disadvantage of this conductive argyle construction is that it can only be fabricated by a relatively complex warp knitting machine, i.e., one having two or more dedicated guidebars as mentioned above.

A need exists, therefore, for a relatively inexpensive easily knitted fabric capable of rapidly and effectively discharging static electricity. Further, the need exists for such a knitted fabric which is capable of discharging static electricity along the course and the wale directions of the fabric and on the technical back and/or face of the fabric. Further, there is also a need for such an antistatic knitted fabric that can be manufactured on a conventional knitting machine that is not as mechanically complex as those required for complex knits, e.g., double argyle, presently used in the industry.

Still further, those environments, particularly hospitals, in which the control of electrostatic charge accumulation is important, require a fabric, including particularly a towel, that can provide a multitude of functions and uses. In addition to control of electrostatic discharge, improved absorbancy, stain resistance and tensile strength, as well as minimized pilling and linting, are important characteristics for fabric, including particularly a towel, used in hospital environments. The advantages of use of this invention in other environments, and in other shapes and forms, are also evident.

Accordingly, it is an object of the present invention to provide a knitted fabric, including particularly a 40 towel, having improved electrical charge dissipation, absorption, stain resistance, anti-pilling and linting and tensile strength properties.

It is a further object of the present invention to provide such a knitted fabric in which an electrostatic charge can be dissipated both along the course direction of the knitted fabric and the wale direction of the knitted fabric on the technical back and/or face.

It is a further object of the present invention to provide a knitted fabric having improved electrical discharge dissipation, absorption, stain resistance, anti-pilling and linting and tensile strength properties in which the percentage of conductive fiber employed in the fabric is significantly less than that required in knitware construction disclosed in the prior art.

It is a still further object of the present invention to provide a knitted fabric that can be manufactured on a conventional knitting machine that is mechanically less complex than those machines presently used to manufacture conductive knitware, i.e., one that requires the use of only one dedicated guidebar.

Other objects and advantages will be in part evident and in part hereinafter pointed out.

#### SUMMARY OF THE INVENTION

In accordance with the above-stated objects a knitted fabric, including particularly a towel, having improved electrical charge dissipation, absorption, stain resis-

tance, anti-pilling and linting, and tensile strength properties is disclosed wherein a series of stitches comprised of nonconductive fibers arranged along the wale direction of the fabric are combined with conductive fibers that form overlaps and underlaps within the nonconductive knit to such an extent so as to form a combined stitch construction, e.g., a modified "Queen's Cord" construction, so that adjacent conductive fibers are in electrical contact providing what is, essentially, an electrically conductive matrix capable of dissipating static charge along substantially any direction of both the course and wale of the fabric, as well as improved absorption, stain resistance, anti-pilling and linting, and tensile strength properties.

15 This invention also provides a method for manufacturing a knitted fabric, particularly in the form of a towel, having improved electrical charge dissipation, absorption, stain resistance, anti-pilling and linting and tensile strength properties comprising the steps of knitting chain stitches of nonconductive fiber along the wale direction with conductive fibers that extend along the course and wale direction and which forms overlaps and underlaps within the nonconductive knit to such an extent so as to form a fabric which is electrically conductive in substantially any direction, and provides improved absorption, stain resistance, anti-pilling and linting and tensile strength properties.

#### BRIEF DESCRIPTION OF THE DRAWING

30 FIG. 1 is a lapping diagram which depicts the stitch formation of the conductive stitch of the present invention.

35 FIG. 2 depicts an enlarged section of the conductive stitch, shown in FIG. 1. This FIG. 2 illustrates the arrangement of the stitches of conductive fiber 1 extending along the course and wale directions and which forms overlaps and underlaps within a nonconductive knit (not shown) so as to form the preferred modified Queen's Cord construction.

40 FIG. 3 depicts a point diagram of Example I.

#### DETAILED DESCRIPTION

Referring to FIG. 1 and FIG. 2, the illustrated sequence of chain stitches may be formed on a knitting machine of the type well known in the art. See, e.g., "An Introduction to the Stitch Formations in Warp Knitting" §1.3, pp. 27-42 (Employees Assoc. Karl Mayer E.V., West Germany 1966) (hereinafter "Stitch Formations") the entirety of which is incorporated herein by reference. A significant advantage of the present invention is that a knitting machine containing only one dedicated guide bar may be employed to fabricate the desired pattern of stitches of nonconductive fiber interlaced with conductive fiber 1.

45 50 55 60 65 66 As illustrated in FIG. 2, the dissipation of electrical charge along both the course and wale directions, as well as improved absorption, stain resistance, anti-pilling and linting and tensile strength properties, are ensured by the novel technique of forming underlaps and/or overlaps with the conductive fiber 1 within a nonconductive knit fabric along both the course and wale directions. This connection of conductive fiber 1 with adjacent nonconductive fibers results in a combined stitch construction, e.g., a modified "Queen's Cord" construction, that is electrically conductive along both the course and wale directions, and, when a two layered knit is fabricated, on both the technical face and back of the fabric. This modified "Queen's Cord" construction

differs from known knit constructions in that the conductive fibers extend either along the course of the fabric or wale of the fabric, unlike the aforementioned argyle pattern in which the conductive fiber extends in a diagonal along the course or wale. "Stitch Formations", at p. 104, FIG. 155, depicts a "Queen's Cord" construction which is to be contrasted with the preferred embodiment of the present invention. It is an important feature of the present invention that the conductive fibers 1 form under and/or overlaps within the nonconductive fabric along the course and wale directions to such an extent that a conductive matrix is formed in which charge can be dissipated along any number of pathways in the course or wale direction of the technical face and back of the fabric.

It is also an important feature of the present invention that the combined stitch construction, e.g., a modified "Queen's Cord" construction, provides absorption characteristics. Still further, the invention demonstrates improved stain resistance and tensile strength, as well as minimizes pilling and linting.

In an alternative embodiment useful, e.g., as an anti-static wall covering, a knitted fabric can be constructed in accordance with the methods of the present invention wherein the conductive fiber is trapped between the overlaps and underlaps of the nonconductive knitted fabric as seen from the technical back.

The conductive fiber 1 can be selected from any of the number of types of conductive fibers commercially available, some of which have been considered in the preceding discussion of the prior art. These conductive fibers can consist either of singular yarns or be plied with other yarns where extra fabric strength or workability is desired.

#### EXAMPLE I

An example of the electrically conductive and absorbant knitted fabric of the present invention, in the form of a towel, was constructed as follows. The bottom bar of an 84 inch Mayer model KC3, 3 bar, 20 gauge warp knit tricot knitting machine was threaded full with 150 denier textured polyester and stitched 45-10. (Idler links for the 3 link per course set-up were omitted in this Example.) The middle bar of the machine was threaded 6 ends out and one end in with 70 denier textured polyester plied with 2 ends per thread of BASF conductive nylon and stitched in the following sequence:

10-10-01-10-01-10-78-78-87-78-87-78-8-7-78.

An intermediate let off was set up for the middle bar on a ratio of 1.21 with a chain sequence as follows:

000(6X444)000-000(6X444)000.

The top bar was threaded 6 ends in and 1 end out with 150 denier textured polyester and stitched 10-01. The knitted fabric so constructed was jet dyed and framed 72 inches wide and slit into 4 separate 18 inch strips. The runner lengths for this fabric were:

top bar: 80 inches per rack

middle bar: 96 inches per rack

bottom bar: 148 inches per rack

The fabric quality pull was 17 inches per rack. The total inches for an 84 inch panel by bar were as follows:

top bar: 2,280 ends

middle bar: 480 ends

bottom bar: 3,360 ends

The fabric was cut into the form of a towel having dimensions of 18" x 33", and the edges of the towel were finished so that the edges do not unravel in normal

wear-and-tear, e.g. with a pearly edge folded small torn edge, a plain serged edge, or by any other means common in the art. The corners of the towel were then squared and sewn.

5 The electrical charge dissipation characteristic of a fabric constructed, in the form of a towel, in accordance with the present invention was tested and is set forth in Example 2.

10 The absorbancy characteristic of a fabric constructed, in the form of a towel, in accordance with the present invention was also tested and is set forth in Example 3.

15 The anti-pilling and linting characteristic of a fabric constructed, in the form of a towel, in accordance with the present invention was also tested and is set forth in Example 4.

20 The stain resistance characteristic of a fabric constructed, in the form of a towel, in accordance with the present invention was also tested and is set forth in Example 5.

25 Still further, the tensile strength characteristic of a fabric constructed, in the form of a towel, in accordance with the present invention was tested and is set forth in Example 6.

#### EXAMPLE 2

30 A sample of antistatic and absorbant fabric, in the form of a towel, and fabricated in accordance with the Example 1 was tested for effective surface resistivity and charge to decay time in accordance with the methods recommended in National Fire Protection Association (NFPA) 99. The tests were conducted at a temperature of 23° C. and a relative humidity of 50%. The fabric measured approximately  $6 \times 10^5$  ohms/cm. in the machine direction and  $2 \times 10^6$  ohms/cm. in the cross-machine direction. Decay times in both directions were much less than 0.01 seconds. The material, therefore, easily met the resistance and decay specifications of National Fire Protection Association (NFPA) Standard 99.

#### EXAMPLE 3

35 A sample of antistatic and absorbant fabric, in the form of a towel, and fabricated in accordance with Example 1 was tested for absorbancy in accordance with the methods recommended in American Association of Textile Chemists and Colorists (AATCC) Standard 79-1986. The test procedure cycle was composed of a 57° C. reverse wheel wash, followed by a tumble dry, 15 minutes autoclave cycle at 121° C., and 15 pounds pressure. After 1, 10 and 50 wash cycles, the fabric demonstrated immediate absorption. The material, therefore, easily met the absorbancy specifications of AATCC 79-1986. The significance of demonstrated immediate absorption after even 50 washings is that the absorbancy derives from the construction of the fabric, is integral in its construction, and is not a factor of any particular finish placed on the fabric. It should further be pointed out that polyester fabrics, while known for 40 stain resistance, anti-pilling and linting, and tensile strength properties, are notoriously hydrophobic.

#### EXAMPLE 4

45 A sample of the antistatic and absorbant fabric, in the form of a towel, and fabricated in accordance with Example 1 was tested for pilling and linting. After 1, 10 and 50 wash cycles, a visual examination of the fabric demonstrated no noticeable pilling and linting.

## EXAMPLE 5

A sample of the antistatic and absorbant fabric, in the form of a towel, and fabricated in accordance with Example 1 was tested for stain resistance in accordance with the methods recommended by an independent testing company. The test procedure involved samples of the fabric that had been washed 1, 10 and 50 times, and then were stained with blood, iodine and surgical jelly. One of each sample was then washed immediately, while another of each sample was allowed to sit undisturbed for 24 hours, after which it was washed. The residual stains, if any, were then rated on a scale from much staining to negligible or no staining. After testing, virtually every sample demonstrated either slight, negligible or no staining.

## EXAMPLE 6

A sample of the antistatic and absorbant fabric, in the form of a towel, and fabricated in accordance with Example 1 was tested for tensile (breaking and tearing) strength in accordance with the methods recommended in American Society for Testing and Materials (ASTM) D-1682 and ASTM D-2661. The tests were conducted at a temperature of 7° C. and a relative humidity of 65%. ASTM D-1682's grab method for testing breaking strength yielded results, in lbs., of 122.6 for wales and 202.4 for courses. ASTM D-2661's tongue tear method for testing tearing strength yielded results, in lbs., of 9.0 for length and 14.4 for width. The material, therefore, easily met the breaking strength and tearing strength specifications of ASTM D-1682 and ASTM D-2661.

It should be understood that this invention's improved electrical charge dissipation, absorption, stain resistance, anti-pilling and linting, and tensile strength characteristics interact to yield the sum of what is this invention.

It should be further understood that this invention is not limited to the illustrations described and shown herein, which are deemed to be merely illustrative of the best modes of carrying out the invention. The invention also encompasses all such modifications which are within the scope of the following claims.

What is claimed is:

1. A knitted fabric having improved electrical charge dissipation, absorption, stain resistance, anti-pilling and linting, and tensile strength properties comprised of stitches of nonconductive fibers knitted together with conductive fibers that form underlaps and overlaps in combination with the nonconductive fibers in both the course and wale directions, the conductive fibers being substantially parallel and perpendicular to the wale of the fabric, so as to form an electrically conductive matrix capable of dissipating charge in substantially any direction along the course and wale of the technical face and back of the fabric.

2. The knitted fabric of claim 1 wherein the conductive fibers are chosen from the group consisting of carbon suffused nylon; filamentary polymer substrates having finely divided, electrically-conductive particles embossed on the fiber surface; and graphite fibers.

3. The knitted fabric of claim 1 wherein the conductive fibers consist of two or more conductive yarns plied together.

4. The knitted fabric of claim 1 wherein the conductive fibers consist of a conductive yarn plied together with a nonconductive yarn.

5. A knitted fabric having improved electrical charge dissipation, absorption, stain resistance, anti-piling and linting, and tensile strength properties, and a modified "Queens Cord" construction fabricated by threaded full the bottom bar of an 84 inch Mayer model KC3, 3 bar, 20 gauge warp knit tricot knitting machine with 150 denier textured polyester stitched 45-10, the middle bar of the machine being threaded 6 ends out and one end in with 70 denier textured polyester plied with 2 ends per thread of BASF conductive nylon and stitched in the following sequence:

10-10-01-10-01-10-01-10-78-78-87-78-87-78-8-

7-78, and with an intermediate let off set up for the middle bar on a ratio of 1.21 and with a chain sequence of:

000(6X444)000-000(6X444)000, and with an intermediate let off set up for the middle bar on a ratio of 1.21 with a chain sequence of:

000(6X444)000-000(6X444)000, and with a top bar threaded 6 ends in and end out with 150 denier textured polyester stitched 10-01.

6. The knitted fabric of claim 1 wherein the conductive fiber is trapped between the overlaps and underlaps of the nonconductive knitted fabric as seen from the technical back.

7. A method of manufacturing a knitted fabric having improved electrical charge dissipation, absorption, stain resistance, anti-pilling and linting and tensile strength properties comprised of knitting stitches of nonconductive fiber together with conductive fibers, the conductive fibers forming overlaps and underlaps with the nonconductive fibers along both the course and the wale directions, the conductive fibers being parallel or perpendicular to the wale of the fabric, thereby forming an electrically conductive matrix capable of dissipating charge in substantially any direction along the course and wale of the technical face and back of the fabric.

8. A method of manufacturing a knitted fabric having improved electrical charge dissipation, absorption, stain resistance, anti-pilling and linting and tensile strength

40 (a) threading full the bottom bar of an 84 inch Mayer model KC3, 3 bar, 20 gauge warp knit tricot knitting machine with 150 denier textured polyester stitched 45-10;

45 (b) threading the middle bar of the machine 6 ends out and one end in with 70 denier textured polyester plied with 2 ends per thread of BASF conductive nylon and stitched in the following sequence: 10-10-01-10-01-10-78-78-87-78-87-78-8-

50 7-78;

(c) setting up an intermediate let off for the middle bar of the machine in a ratio of 1.21 with a chain sequence of:

000(6X444)000-000(6X444)000;

55 (d) threading the top bar of the machine 6 ends in and 1 end out with 150 denier textured polyester stitched 10-01.

9. A towel comprised of stitches of nonconductive fibers knitted together with conductive fibers that form underlaps and overlaps in combination with the nonconductive fibers in both the course and wale directions, the conductive fibers being substantially parallel and perpendicular to the wale of the fabric, so as to form an electrically conductive matrix capable of dissipating charge in substantially any direction along the course and wale of the technical face and back of the towel.

60 10. A method of manufacturing a towel having improved electrical charge dissipation, absorption, stain

resistance, anti-pilling and linting and tensile strength properties comprised of knitting stitches of nonconductive fiber together with conductive fibers, the conductive fibers forming overlaps and underlaps with the nonconductive fibers along both the course and the wale directions, the conductive fibers being parallel or perpendicular to the wale of the fabric, thereby forming an electrically conductive matrix capable of dissipating charge in substantially any direction along the course and wale of the technical face and back of the towel.

10 11. A method of manufacturing a towel, having improved electrical charge dissipation, absorption, stain resistance, anti-pilling and linting and tensile strength properties, and a modified Queen's Cord construction comprising:

- (a) threading full the bottom bar of an 84 inch Mayer model KC3, 3 bar, 20 gauge warp knit tricot knitting machine with 150 denier textured polyester stitched 45-10;
- (b) threading the middle bar of the machine 6 ends 20 out and one end in with 70 denier textured polyesters.

ter plied with 2 ends per thread of BASF conductive nylon and stitched in the following sequence: 10-10-01-10-01-10-01-10-78-78-87-78-87-8-8-7-78;

(c) setting up an intermediate let off for the middle bar of the machine in ratio of 1.21 with a chain sequence of:

000(6X444)000-000(6X444)000;

(d) threading the top bar of the machine 6 ends in and 1 end out with 150 denier textured polyester stitched 10-01.

(e) Trimming the fabric into the shape of a towel having dimensions of 18" X 33".

(f) Finishing the edges of the fabric so that it does not unravel in normal wear-and-tear, e.g. with a pearl edge folded, small turn edge, plain serged edge, or by any other means common in the art.

(g) Squaring the corners of the fabric by sewing or by any other means common in the art.

\* \* \* \* \*

UNITED STATES PATENT AND TRADEMARK OFFICE  
CERTIFICATE OF CORRECTION

PATENT NO. : 4,856,299

DATED : August 15, 1989

INVENTOR(S) : Kenneth G. Bryant

It is certified that error appears in the above-identified patent and that said Letters Patent is hereby corrected as shown below:

Column 3, line 48, change "and/or" to --and--;

Column 8, line 4, change "threaded" to --threading--;

Column 8, line 20, delete "and end" and insert --and one end--;

Column 8, line 40, after "strength" insert --properties, and a modified Queen's Cord construction comprising:--

Column 9, line 6, delete "or" and insert --and/or--;

Signed and Sealed this  
Seventh Day of August, 1990

*Attest:*

HARRY F. MANBECK, JR.

*Attesting Officer*

*Commissioner of Patents and Trademarks*